

Nov. 30, 1943.

E. J. BALLINTINE ET AL

2,335,376

PROCESS OF MANUFACTURING MULTIPLE GLAZED UNITS

Filed Feb. 27, 1941

Fig. 1.



Fig. 2.



Fig. 3.



Inventors  
ELMER J. BALLINTINE and  
FRANK F. PAINTER

By

Olen E. Bee  
Attorney

## UNITED STATES PATENT OFFICE

2,335,376

PROCESS OF MANUFACTURING MULTIPLE  
GLAZED UNITSElmer J. Ballantine and Frank F. Painter,  
Tarentum, Pa., assignors to Pittsburgh Plate  
Glass Company, a corporation of Pennsylvania

Application February 27, 1941, Serial No. 380,760

2 Claims. (Cl. 154—28)

The present invention relates to insulating structures and more particularly to a process of manufacturing multiple glazed units.

One object of the invention is to provide a process in which hermetically sealed multiple glazed units are readily obtained.

A second object of the invention is to provide a process wherein a metallic seal of high mechanical strength is developed for a multiple glazed unit.

Other objects and advantages of our invention will become more readily apparent from the following detailed description of certain preferred embodiments thereof.

Multiple glazing units are becoming of increasing importance to the building industry, especially since air-conditioning has been so widely adopted. The insulation value of these multiple glazed units results from their enclosed air spaces. It will at once be apparent that the units should be hermetically sealed to prevent infiltration of moisture or foreign matter into the units.

We are aware that various means of sealing multiple glazed units have been advanced heretofore. A vitreous seal is disclosed in U. S. Patent No. 2,032,003, issued February 25, 1936, to R. L. Clause, and a metal seal is the subject matter of U. S. Patent No. 2,198,578, issued April 23, 1940, to B. F. Hazelton. It is believed, however, that a more permanent union between spaced glass plates can be obtained in a more facile manner. Briefly stated, the present invention contemplates the application to the glass plates of a metallic glaze to which the vapor barrier or other sealing means is secured.

In the drawing:

Figure 1 is an elevational view of a multiple glazed unit embodying the principles of our invention;

Figure 2 is a fragmentary vertical sectional view thereof; and

Figure 3 is a fragmentary vertical sectional view of another form of the invention.

Referring to the drawing, a multiple glazed unit 2 comprises glass plates 3, having marginal coatings 5 of an electrical conducting glaze fused thereon, arranged in parallel relation with the glazed portions in register and held apart by a spacer 7 which is secured to the glazed portions.

Another form of the invention is illustrated in Figure 3 wherein a multiple glazed unit 11 comprises a plurality of glass plates 12, having marginal coatings 14 of an electrical conducting glaze fused thereon and covered with films 15 of electrolytically deposited copper, arranged in parallel

relation with the glazed portions to the outside and held apart by a spacer 17 of resilient material, such as rubber, synthetic resin, etc. A strip 19 of metal substantially of U-shape in cross-section is fitted over the edges of the glass plates and secured to the glazed portions thereof.

The electrical conducting glaze which coats the margins of the glass plates comprises fine particles of silver, colloidal silver, admixed with 10 lead borate, a boro silicate, or other fusible glaze in a ratio of from 2 parts metal to 1 part of glaze to 8 parts of metal to 1 part of glaze. This ratio may be varied as desired within these limits, it being necessary only to maintain sufficient metal 15 in the mixture that it remains electrical conducting. The mixture may be combined with a suitable vehicle, such as turpentine, oil of violet, linseed oil, and a binder of brown sugar, molasses or the like, to facilitate application to the glass plates and subsequent handling. Gold or platinum may be substituted for the silver of the glaze, although the cost factor will generally preclude this substitution. Nickel is another example of a metal which may be included in the glaze coating.

The glazing mixture is applied to the margins of glass plates in a uniform coating and the plates are heated to fuse the glaze and bond or weld the coating to the glass. This operation 20 may be carried out in a continuous process by passing the sheets through a kiln which is heated to give a gradually increasing temperature to fuse the glaze in the forepart and cooled gradually thereafter to reduce the temperature of the 25 plates to normal.

In assembling the unit, as shown in Figures 1 and 2, the glazed portions of the plates are tinned and given a thin coating of ordinary or silver solder. The spacer 7, which is of metal, 30 is likewise tinned and coated with solder. The glazed plates are arranged in parallel relation with the glazed portions in register and with the spacer therebetween. On heating the assembly, the solder melts and creates a bond between the spacer and the glaze, thus sealing the edges of the unit.

In the form of our invention, shown in Figure 3, the plates, after the glaze has been fused thereon, are submerged in a copper sulfate solution and a film of copper is deposited electrolytically over the glaze. The metal content of the glaze permits this operation without difficulty. The coated glaze is tinned and covered with solder as before.

The plates are assembled in parallel relation

with the glazed portions exposed and held apart by a spacer of rubber or other resilient material. A channel strip of metal substantially of U-shape in cross-section is fitted over the edges of the assembly and sufficient heat is applied thereto to melt the solder and thus seal the metal strip to the copper plated glaze.

Due to the fact that solder is employed to create the bond and seal of the unit, negligible pressure changes are experienced in the air space 10 between the glass plates. Accordingly a complete edge seal may be provided in the first instance which will not rupture on cooling.

It will at once be obvious that various modifications in the several elements of our construction and their combination are possible without departing from the spirit of the invention or the scope of the appended claims.

What we claim is:

1. A process of manufacturing a multiple 20 glazed unit which comprises coating marginal

portions of glass plates with an admixture of metal and vitreous material thereby forming electrical conducting films on said plates, heating the plates and films sufficiently to fuse the plates and films together, electrolytically depositing a layer of copper on said films, assembling the plates in parallel spaced relation, and securing a vapor barrier to the copper layers to seal in the space between the plates.

2. A process of manufacturing a multiple glazed unit which comprises coating marginal portions of glass plates with colloidal metal admixed with a fusible vitreous material thereby forming a fusible glaze on the glass, fusing the glaze and glass together, assembling the glass plates in spaced parallel relation, and soldering a metal vapor barrier to the glaze to seal in the space between the plates.

ELMER J. BALLINTINE.  
FRANK F. PAINTER.